

April 5, 1938.

H. NEUMANN

2,112,971

FERROMAGNETIC ALLOY

Filed Oct. 20, 1934



Invantor  
Hans Neumann  
by Knight, Bray attorney

## UNITED STATES PATENT OFFICE

2,112,971

## FERROMAGNETIC ALLOY

Hans Neumann, Berlin-Siemensstadt, Germany,  
assignor to Siemens & Halske, Aktiengesellschaft,  
Siemensstadt, near Berlin, Germany, a  
corporation of Germany

Application October 20, 1934, Serial No. 749,163  
In Germany October 24, 1933

4 Claims. (Cl. 148—31)

My invention relates to ferromagnetic alloys containing principally iron, nickel and copper. As to the nature of such alloys it is well known that certain compositions are characterized by a high permeability, others by a small coercive force.

According to the present invention permeable ferromagnetic alloys containing as essential constituents iron, nickel and copper are so chosen that the composition as to the content of the three above-mentioned constituents lies within a definite range, characterized in the accompanying composition diagram by the hatched area. In this case the final, quaternary alloy must, besides, contain still an amount of molybdenum greater than 1 per cent, but not more than 10 per cent. Thus, in all cases the final product is a quaternary alloy. As will be apparent from the diagram of the drawing in the case of alloys containing molybdenum ternary master alloys are employed which contain at most 25 per cent iron, at most 55 per cent copper and 40 to 90 per cent nickel.

With alloys thus composed not only is it possible to attain particularly high initial permeabilities, but also the alloys have at the same time the advantage that the maximum permeability coincides with the minimum coercive force.

It is well known in the art to add molybdenum to ferromagnetic alloys. Thus, for instance, a small amount of molybdenum has been hitherto added to iron-nickel alloys so as to increase the specific resistance. However, in these alloys the initial permeability is not increased by the molybdenum content. Further, the value of the coercive force remains relatively high, i. e., the values obtained are all greater than  $H_c = .035$  Oersted.

If an amount of molybdenum of not less than 1 and not more than 10 per cent is, however, added according to the invention to iron-nickel-copper alloys containing 40 to 90 per cent nickel and not more than 25 per cent iron with not more than 55 per cent copper, considerably higher initial permeabilities and smaller coercive forces may be attained.

Favorable results are obtained, if the composition of the alloys is so chosen that the composition as to its iron-, nickel-copper content lies within the hatched range as shown in the accompanying diagram. In this diagram for the Fe element content the abscissa is represented by the line Cu—Ni, and the ordinate by the line Cu—Fe; for the Ni content the abscissa line is Fe—Cu, the ordinate line Fe—Ni, and for the Cu content the abscissa line is Ni—Fe, and the

ordinate line Ni—Cu. In all cases where in this shaded area the constituents of the ternary master alloy supplement one another to 100%, the content of at least one of the three constituents is assumed to be reduced percentually to the extent to which molybdenum is added, so that the content percentages of the final, quaternary alloy total up 100%. Thus, for instance, in an alloy lying within this range containing 70 per cent nickel, 13 per cent iron and 17 per cent copper, an initial permeability  $\mu_0 = 18,000$  may be attained. However, if a composition of 70 per cent nickel, 10 per cent iron, 17 per cent copper and 3 per cent molybdenum is chosen according to the invention the value of the initial permeability may be increased to  $\mu_0 = 25,000$ .

While with iron-nickel-copper alloys free of molybdenum initial permeabilities of about 18,000 are obtained, such alloys containing molybdenum may have an initial permeability exceeding double the amount. For instance, initial permeabilities of more than 40,000 have been obtained, the coercive force being at the same time reduced. More exact values are indicated in the following table which shows a comparison of iron-nickel-copper alloys without and with molybdenum.

| NI | Cu | Fe | Mo | Percentage of |       | Character of alloy   | Resistance in ohm/m/mm <sup>2</sup> |
|----|----|----|----|---------------|-------|----------------------|-------------------------------------|
|    |    |    |    | $\mu_0$       | $H_c$ |                      |                                     |
| 70 | 17 | 13 | —  | 18000         | .026  | 100% ternary.....    | .32                                 |
| 70 | 17 | 10 | 3  | 25000         | .0126 | 100% quaternary..... | .57                                 |
| 72 | 14 | 14 | —  | 13250         | .068  | 100% ternary.....    | .31                                 |
| 72 | 14 | 11 | 3  | 49000         | .014  | 100% quaternary..... | .56                                 |

In this case the alloys free of molybdenum upon exposing them to the air are suddenly cooled, whereas the alloys containing molybdenum are gradually cooled in the furnace. This difference in treatment will be presently described.

As will be apparent from the above table, besides the high initial permeability, coercive forces lying between .01 and .02, i. e., considerably lower than the optimum values hitherto attained in ferromagnetic alloys may be obtained with alloys according to the invention. Such low values have been hitherto only obtained with pure iron in the research laboratory. However, it was not possible to utilize these favorable values technically, since it is difficult to produce iron of sufficient purity in great quantities economically. Furthermore, it is practically impossible to maintain the iron pure when subjecting it to the treatment required, whereas the production

and treatment of ferromagnetic alloys according to the invention present no difficulties. Furthermore, also the value of the specific resistance simultaneously attained with the low coercive force is considerably greater and, therefore, more favorable than in the case of pure iron.

As a result of the small coercive force the material according to the invention becomes extremely important, for instance, for the manufacture of relays which owing to the great reduction of the interfering coercive force may be considerably simplified. The manufacture of magnetic bodies may also be greatly improved owing to the following circumstance: In iron-nickel-copper alloys free of molybdenum the maximum initial permeability is obtained by cooling the alloys suddenly from a higher temperature. The addition of molybdenum has the effect that the favorable magnetic properties are obtained by a gradual cooling. The material is, for instance, kept for 5 to 10 hours at an annealing temperature of about 1100° C. and then it is gradually cooled in the furnace. By avoiding a sudden cooling of the material not only the pro-

duction of magnetic bodies is simplified but it also eliminates the danger that stresses due to chilling may occur in the body which impair its magnetical properties.

The addition of molybdenum has not only the effect of increasing the permeability of the alloy, but also the specific resistance as is apparent from the above table.

I claim as my invention:

1. A highly permeable ferromagnetic alloy consisting of 72% Ni, 14% Cu, 11% Fe and 3% Mo.
2. A highly permeable ferromagnetic alloy consisting of 70% Ni, 17% Cu, 10% Fe and 3% Mo.
3. A highly permeable ferromagnetic alloy consisting of 70-74% Ni, about 10-12% Fe, 2-4% Mo and the rest copper.
4. A highly permeable ferromagnetic material consisting of 70-74% Ni, about 10-12% Fe, 2-4% Mo and the rest copper, and having an enhanced initial permeability obtained by annealing at 600 to 1100° C. and then gradually cooling the material.

HANS NEUMANN.